

# UNITED STATES PATENT OFFICE.

MAX MÜLLER, OF ALTDAMM, GERMANY.

## PROCESS OF PRODUCING LUSTROUS THREADS, &c., FROM VISCOSE.

No. 836,452.

Specification of Letters Patent.

Patented Nov. 20, 1906.

Application filed April 24, 1906. Serial No. 813,511.

*To all whom it may concern:*

Be it known that I, MAX MÜLLER, a subject of the King of Prussia, German Emperor, residing in Altdamm, Prussia, Germany, have invented certain new and useful Improvements in Processes of Producing Lustrous Threads, Bands, Strips, &c., from Viscose, of which the following is a specification.

10 My invention relates to the method of producing lustrous threads and the like from viscose solution.

It is known that lustrous threads or the like can be produced from viscose—for example, as described in the German Patent No. 70,999—if it is permitted to pass out of suitably-formed openings into a solution of sulfate of ammonia or into acids.

When using sulfuric acid for the purpose indicated, it is shown that diluted acid acts but slowly, and the water present gives a slimy constitution to the thread or film, which on working farther up causes great loss in material. If the action of diluted acid is supported by heat, the thread does indeed become firmer and is more easily worked; but as the gaseous products of decomposition of the viscose solution—for example, hydrosulfuric acid, carbonic acid—are almost insoluble, or at all events soluble with difficulty, in warm liquid, they escape as gases and occasionally pass as small bubbles through the sides of the tube of cellulose hydrate, which represents the first stage of thread formation. A long series of experiments, in which sulfuric acid of varying concentration (containing between five per cent. and forty per cent. of sulfuric acid) was employed, show that all the threads produced when microscopically examined no longer have a smooth structure provided with some longitudinal strips, but show a slight similarity to a thread which is thickly covered with fine scales.

45 Concentrated sulfuric acid acts on the viscose solution in quite similar manner. Here the gaseous products escape for want of a solvent, and the formation of a lustrous thread or the like is entirely thwarted; but if the sulfuric acid is diluted so far as the disturbing development of gas is avoided, and if at the same time the softening action of the diluting-water on the thread in process of formation is counterbalanced by adding a suitable 50 quantity of salt, a product of conspicuous qualities in regard to strength, luster, and

elasticity is obtained. All soluble sulfates, including those of the heavy metals, are suitable, and naturally also all those salts and oxids or elements which when in contact with 60 sulfuric acid turn into sulfates.

A very suitable precipitating-bath is obtained, for example, if forty kilograms bisulfate of sodium be dissolved in sixty kilograms of water and seven kilograms of sulfuric acid, sixty-six per cent., be added. The acid concentration corresponds to about twenty per cent.

The sulfates *per se* without addition of acid are not suited to the production of shiny 70 structures of cellulose hydrate from viscose solution, excepting only sulfate of ammonia, which changes the viscose at once into cellulose xanthogenate of ammonia, which is at once further decomposed, with separation of 75 cellulose hydrate. As the viscose solutions possess a high percentage of free soda, it is inevitable that almost the entire ammonia escapes in the form of gas, especially as the precipitation solutions must 80 be employed at a higher temperature. That process, because of the high commercial value of ammonia, is therefore essentially more expensive through the losses or through the costly apparatus for regaining the same. 85

Other sulfates are not suited for the present purpose, for some—as, for instance, sulfate of zinc or sulfate of magnesia when in viscose solution—through reciprocal decomposition yield insoluble salts of cellulose 90 thiocarbonic acid, from which cellulose hydrate can be separated only through further suitable action. The others, such as sulfate of potassium or of sodium, simply precipitate viscoses which are insoluble in salt solutions 95 and only the further treatment of the viscose and salt solution by chemical agencies or heat can bring about the formation of cellulose hydrate. For instance, one does not succeed with the most concentrated sulfate 100 of soda in producing lustrous threads from viscose solutions. On the other hand, the precipitating-bath just described, composed of solution of bisulfate of sodium and sulfuric acid, is well suited for the purpose, even at 105 room temperature. The slight commercial value of the materials employed and the fact that bisulfate sulfuric acid and caustic soda are easily useful in the form of sulfate of soda calculated to assure for the bisulfate 110 process precedence as compared with the employment of sulfate of ammonia.

In order to obtain the very shiny product decomposition of the viscose aimed at by the process in the form of threads, bands, &c., the sufficiently purified and concentrated viscose solution is permitted to pass out of suitably-formed openings into a solution of the composition described, and the separated cellulose hydrate is collected by winding it onto spools or reels or in any other manner in order to bring it into convenient form to be further worked up.

What I claim as my invention, and desire to secure by Letters Patent, is—

1. The method of producing threads of the character described consisting of permitting the viscose solution to pass out through suitably-formed openings into a precipitating-bath containing sulfuric acid and a salt.
2. The method of producing threads of the character described consisting of permitting the viscose solution to pass out of suitably-formed openings into a precipitating-bath

containing sulfuric acid and a soluble sulfate salt.

3. The method of producing threads of the character described consisting of permitting the viscose solution to pass out of suitably-formed openings into a precipitating-bath, containing sulfuric acid and bisulfate of sodium.

4. The method of producing threads of the character described consisting of permitting the viscose solution to pass out of suitably-formed openings into a precipitating-bath containing sulfuric acid and bisulfate of sodium, and water in the proportions substantially as specified.

In testimony whereof I have signed my name to this specification in the presence of two subscribing witnesses.

MAX MÜLLER.

Witnesses:

WILH. GRIESKE.

HANS HILDEBRAND.